

## UNITED STATES PATENT OFFICE

HANS SIMON, OF HANOVER, GERMANY, ASSIGNOR TO GUNTHER WAGNER, OF HANOVER, GERMANY, A CORPORATION OF GERMANY

## DUPLICATING STENCIL

No Drawing. Application filed June 15, 1931, Serial No. 544,701, and in Germany April 20, 1931.

This invention relates to improvements in duplicating stencils and a method for producing the same.

It has been known to use, as a duplicating stencil, a fibrous and porous Japanese paper coated with a layer of hardened or non-hardened proteins to which softening agents such as glycerine, sugar, fats, fatty acids, etc. have been added. Such duplicating stencils have, however, the drawback that the softening agent added to the proteins is liable, during the storage of the stencil, to be exuded at the surface of the coating in such quantities that the stencil will become sticky and consequently useless. It is not possible to eliminate this drawback by diminishing the amount of the softening agents added to the proteins because a certain amount of said softeners is required to keep the coating plastic. If the amount of the softeners added to the proteins is less than a certain positive value, the coating will become hard and full of cracks after a certain period of storage, so that it will be impractical to use it. Nor is it possible to eliminate completely this precipitation of softeners in the coating by mixing inorganic fillers therewith, consisting, for instance, of bentonit or kaolin, as has been proposed in prior art, because such pastes cannot prevent, with certainty, this exudation for a sufficiently long time.

The main object of this invention is to eliminate the above-mentioned drawback and to provide a duplicating stencil which can be safely stored for a considerable period of time and which has a coating that remains soft and plastic during this storage.

A further object of this invention is to provide a stencil coating comprising proteins and softeners mixed with substances by means of which said softeners may be equally distributed in the coating and securely bound therewith.

A still further object of this invention is to provide a duplicating stencil for type-

writing and duplicating machines, which will not smear the types or grease and dirty the caoutchouc rollers of said machines.

The above-mentioned objects can be realized by adding organic fillers as distinguished from inorganic fillers heretofore used, to the coating, such organic fillers consisting, for instance, of a very finely ground wood-flour, such as beechwood (*Fagus sylvatica*) or bamboo-wood (*Arundo bambos*), or of horn-dust, *Lycopodium* dust or other substances.

Horn dust is derived by powdering or grinding the horn material of animals, while *Lycopodium* dust (lycopode) is a yellow powder derived from the spores of the club moss, especially *L. clavatum*, *L. selago*, *L. phlegmatis*, *L. rubrum*, *L. saussurus*, etc.

An organic filler of this kind will effectively bind the softeners within the coating and will further the even distribution of such softeners. Duplicating stencils provided with a coating in accordance with this invention remain uniformly soft and flexible even after having been stored for a very long time and the precipitation of softeners is totally prevented. This is not the case with duplicating stencils provided with a protein coating as known in prior art, which become sticky after a certain period of storage or hard when the coating does not contain a sufficient amount of softeners.

A further advantage of adding an organic paste to the stencil coating resides in the fact that when the duplicating stencil is used in connection with a typewriter the types will not become dirty or blocked. Furthermore, the softeners forming part of the coating and consisting of oils or fats will not be deposited on the rubber rollers of the typewriters and duplicating mechanisms.

I have found that the best results are obtained when an organic filler consisting of a wood-dust is added to the coating substance and used in connection with other substances.

An example of a mixture which may be employed is as follows:

|                                                                                                       | Parts by weight |
|-------------------------------------------------------------------------------------------------------|-----------------|
| 5 Gelatine                                                                                            | 10              |
| 5 Glycerine                                                                                           | 3               |
| 10 A sulphonated animal or vegetal oily matter, for instance, sulphonated castor-oil (Turkey red-oil) | 18              |
| 10 Petroleum jelly                                                                                    | 60              |
| 10 Castor oil                                                                                         | 2               |
| 10 Olive oil                                                                                          | 2               |
| 10 Beechwood dust                                                                                     | 10              |
| 10 Methylene blue                                                                                     | .75             |
| 15 Sodium p-chlorbenzoate                                                                             | .35             |
| 15 Water                                                                                              | 200             |

This liquid mixture is applied in the usual way onto a sheet of Japanese paper at the usual temperature of about 50° C. and is dried 20 then at the same temperature so that the water evaporates.

The advantageous results obtained from the use of organic fillers, such as wood flour, are achieved owing to the fact that the wood-dust comprises a certain small amount of 25 coagulating or tanning substances which have a slight hardening effect on the proteins contained in the coating substance.

It is possible to increase the hardening 30 effect by adding another substance, for instance, a formaldehyde, to the coating.

I claim:

1. A process for manufacturing duplicating stencils, comprising the steps of adding 35 a substantially insoluble organic filler to a coating mixture containing proteins and softening agents, and then applying said coating mixture onto a fibrous and porous sheet.

40 2. A process for manufacturing duplicating stencils, comprising the steps of adding a wood-dust to a coating mixture containing proteins and softening agents, and then applying said coating mixture onto a fibrous and porous sheet.

45 3. A process for manufacturing duplicating stencils, comprising the steps of adding horn-dust to a coating mixture containing proteins and softening agents, and then applying said coating mixture onto a fibrous and porous sheet.

50 4. A process for manufacturing duplicating stencils, comprising the steps of adding Lycopodium dust to a coating mixture containing proteins and softening agents, and then applying said coating mixture onto a fibrous and porous sheet.

55 5. A process for manufacturing duplicating stencils, comprising the steps of adding a substantially insoluble organic filler to a coating mixture containing proteins and softening agents, then adding a hardening agent to the mixture, and then applying said coating mixture onto a fibrous and porous sheet.

60 6. A process for manufacturing duplicat-

ing stencils, comprising the steps of adding a substantially insoluble organic filler to a coating mixture containing proteins and softening agents then adding a formaldehyde to the mixture, and then applying said coating 70 mixture onto a fibrous and porous sheet.

7. A coating for duplicating stencils, comprising a mixture of petroleum jelly, a sulphonated non-mineral oil, gelatine, a wood-dust, glycerine, castor oil, olive oil, methylene 75 blue and sodium para-chlorbenzoate.

8. A coating for duplicating stencils comprising, 60 parts by weight of petroleum jelly, 18 parts by weight of a sulphonated non-mineral oil, 10 parts by weight of gelatine glue, 10 parts by weight of a wood-dust, 3 parts by weight of glycerine, 2 parts by weight of castor oil, 2 parts by weight of olive oil, .75 part by weight of methylene blue and .35 part by weight of sodium para-chlorbenzoate. 80

9. A coating for duplicating stencils comprising a mixture of hardened gelatin, a softening agent and a permanent finely divided substantially insoluble organic filler. 85

10. A coating for duplicating stencils comprising a mixture of hardened gelatin, a softening agent and a powdered organic filler containing small quantities of a tanning material. 90

11. A coating for duplicating stencils comprising a mixture of hardened gelatin, a softening agent and a powdered cellulose filler. 95

100 12. A coating for duplicating stencils comprising a mixture of hardened gelatin, a softening agent and one of a group of powdered organic fillers, said group including beechwood flour and bamboo wood flour.

In testimony whereof I have affixed my 105 signature.

HANS SIMON.

110

115

120

125

130